

April 27, 1954

M. H. EDSON

**2,676,910**

## PROCESS FOR PRODUCING AND REFINING ASPHALT

Filed May 26, 1951



## UNITED STATES PATENT OFFICE

2,676,910

PROCESS FOR PRODUCING AND REFINING  
ASPHALTMurray H. Edson, Roselle, N. J., assignor to  
Standard Oil Development Company, a corpora-  
tion of Delaware

Application May 26, 1951, Serial No. 228,499

5 Claims. (Cl. 196—74)

1

This invention concerns a novel process for treating residual oils and hydrocarbon residues, to obtain asphalts of desirable properties. The process employed depends upon a heat treatment of the residual oil in the presence of  $P_2O_5$ . This process can in many cases be advantageously varied by air blowing the residual oil prior to contact with  $P_2O_5$ , or by air blowing the asphalt obtained by treatment of residual oil with  $P_2O_5$ . While as indicated, the process is particularly 10 adapted for the treatment of residual oils to recover asphalts therefrom; the process may also be employed for the upgrading of asphalts obtained by conventional processing steps.

The present invention concerns the recovery 15 of asphalts and the refining of asphalts obtained from petroleum oils. The principal objective of the process herein disclosed is to provide asphalts having unusual properties; in particular, asphalts are obtained which have usually high penetration and ductility properties for a given softening point, although, as will be brought out, other desirable properties may also be realized. This unusual combination of characteristics is demanded in a number of applications, an outstanding example of which is the lining of irrigation canals. Asphalts employed to line irrigation canals ideally should have properties to enable the asphalt lining to retain its shape in hot weather, to be non-brittle in cold weather, and to conform to the contour of the surface of the canal without tearing. Asphalts having these properties must have a softening point of about 175° to 200° F., and must have high ductility and high values of penetration. It has been found that asphalts obtained by conventional processing methods do not have the necessary combination of properties. More precisely, the asphalts obtained by conventional processing techniques, in the range of softening points identified, have too low a ductility and too low a penetration to meet the desired characteristics.

It is therefore the principal object of this invention to provide an asphalt recovery and treating process which will vary the usual combination of softening point, penetration, and ductility properties. To bring out the manner in which these asphalt properties are affected, it is helpful to consider the results of subjecting crude residua to an oxidation treatment as achieved by conventional air blowing. Oxidation treatments of this character are well known to the art and it has been appreciated that the low temperature susceptibility of asphalts may to some extent be improved by oxidation. However, when air blowing is applied and continued, while the softening point of an asphalt is raised, the penetration is decreased and the ductility is

5 20

lowered. Consequently, contra to this change in asphalt properties, the process of this invention provides an increase in penetration properties and an increase in ductility concomitant with the increase in softening point of the asphalt.

The process by which these desirable changes in asphalt properties are obtained depends upon the catalytic treatment of residual oils or asphalts with  $P_2O_5$ . The precise mechanism of the asphalt change which occurs is not understood, although the principal effect appears to depend upon polymerization and condensation reactions. It is important to note that the treatment is in no respect an oxidation treatment, and in fact oxidation or the presence of air during the process is to be avoided. Thus, it has been determined that for the purposes of this invention, degradation in asphalt quality results from the presence of air during treatment with the  $P_2O_5$ .

25 The quantity of  $P_2O_5$  to be employed ranges from about 0.1 to 5% by weight. The precise amount of  $P_2O_5$  to be used depends principally upon the properties desired and the starting materials. In all cases treatment with  $P_2O_5$  is preferably continued until equilibrium has been obtained. As the  $P_2O_5$  treatment of asphalt proceeds readily, the time required is reasonably short and does not ordinarily exceed one hour. The temperature of treatment with  $P_2O_5$  is chosen from the range of 300° to 550° F. Again, the precise temperature to be used depends to some extent upon the asphalt characteristics desired and the starting materials.

30 35 40 This treatment of a residual oil or an asphalt with  $P_2O_5$  at 300° to 550° F. in the absence of air or oxygen produces a material change in the properties of the asphalt. In particular, the softening point of the asphalt is raised and the temperature susceptibility of the asphalt is improved to values otherwise unobtainable.

45 50 55 While as indicated, the critical treatment with  $P_2O_5$  depends upon the exclusion of any oxidation effects, it has been found valuable in certain applications to employ an oxidation treatment either before or after, but not simultaneously with the  $P_2O_5$  treatment. One adaptation of the process of this invention therefore depends upon oxidizing an asphalt followed with  $P_2O_5$  treatment in the absence of air; another adaptation of the process utilizes  $P_2O_5$  treatment in the absence of air followed by an oxidation treatment. Both of these adaptations causes a variation in asphalt properties different from those which occur without the oxidation treatment or when the oxidation is applied simultaneously with the  $P_2O_5$  treatment. Furthermore, the oxidation treatment when applied before or after

the  $P_2O_5$  treatment, decreases the amount of  $P_2O_5$  required to attain a particular softening point.

To fully disclose the nature of this invention, reference will be made to the accompanying drawing which diagrammatically illustrates a flow plan of a preferred process embodying this invention. The process illustrated in the drawing concerns the preparation of asphalt from a residual oil obtained by distillation of a crude petroleum oil, although it is to be understood that the process illustrated may be applied to asphalts which may be obtained by other methods. The term "residual oils" by definition is employed to identify the liquid or semi-solid residues obtained from the destructive distillation of non-asphaltic petroleum, from the distillation of semi-asphaltic and asphaltic petroleums, from the distillation of pressure tar, or from the fluxing of harder residual asphalts with heavy distillates. The term "flux" or "flux oil" may be used synonymously with the term "residual oil."

By way of example, in the process illustrated in the drawing, a residual oil is obtained in distillation zone 1 by treatment of a semi-asphaltic or asphaltic petroleum oil introduced to still 1 through line 2. Normally gaseous hydrocarbons may be withdrawn from distillation zone 1 through line 3, while side stream products consisting of gasoline, kerosene, gas oil, lubricating oil, etc., may be withdrawn through lines 4, 5, 6, etc. The residual oil may be removed as the bottoms produced from the distillation zone through line 7 and will include substantially all of the asphaltic constituents originally present in the crude oil distilled. The specific gravity of the residual oil at 77° F. will range from about 0.85 to 1.07, and the fusing point of the oil as determined by the ring and ball method will generally fall within the range of 32° to 120° F. This residual oil may be converted to an asphalt of desirable properties by the processing sequence illustrated in the drawing.

As will be brought out, the primary and essential treatment of the residual oil depends upon a catalytic treatment with  $P_2O_5$  in refining zone 10. Use of the two air blowing zones 11 and 12 is optional and for simplicity it may be assumed that zones 11 and 12 are by-passed by the by-pass lines provided. In this case the residual oil withdrawn from distillation zone 1 through line 7 will preferably be passed through a pre-heater 13 and will then be introduced directly into refining zone 10. Sufficient  $P_2O_5$  is introduced to zone 10 through line 14 to provide a weight percent of about 0.1 to 5%. Mechanical agitation by inert gases such as nitrogen is employed in zone 10 to thoroughly mix the residual oil and  $P_2O_5$ . By suitably preheating the residual oil in preheater 13 and/or by utilizing heating jackets, steam coils, etc., in zone 10, mixing in zone 10 is carried out at a temperature in the range of 300° to 550° F. Care is taken to exclude air or oxygen from zone 10. As a result, with this treatment of  $P_2O_5$ , the softening point of the asphalt is increased and other properties of the asphalt are changed. The ultimate properties obtainable are dependent upon the particular temperature of treatment, the percentage of  $P_2O_5$  employed, and the initial flux oil treated. Prior to reaching equilibrium properties, the time of treatment will also affect the asphalt properties. However, it is important to continue the mixing until no further change in properties occurs. This can

75  
1 Penetration temperature susceptibility =

$$\log 800 - \log \text{pen. at } 77^\circ \text{ F.} \\ \text{softening point } (^\circ \text{ F.}) - 77$$

be readily determined by periodically determining the softening point, the penetration or other inspections of the asphalt during treatment. In general, about 30 to 90 minutes are to be employed for the  $P_2O_5$  treatment, depending upon starting material, temperature, quantity of change, amount of  $P_2O_5$ , and degree of agitation. The final asphalt product may then be removed from zone 10 through line 15.

As will be demonstrated, in some cases it is preferred to air blow the residual oil or asphalt prior to the  $P_2O_5$  treatment. In this case the residual oil of line 7 is introduced to zone 11 for contact with an oxidation agent such as air. The oxidation treatment may be conducted in any desired manner; for example, by blowing about 30 to 50 cu. ft. of air per minute per ton of asphalt through the residual oil at about 300 to 550 F. temperature. Thereafter the air blown oil may be withdrawn from zone 11 and passed through preheater 13 for treatment with  $P_2O_5$  in zone 10 as described. The final asphalt product is then obtained by withdrawing the asphalt directly from zone 10 through line 15.

Rather than applying the oxidation treatment prior to  $P_2O_5$  treatment, it is sometimes preferred to apply the oxidation treatment after the  $P_2O_5$  treatment. In this case the residual oil of line 7 will by-pass zone 11 and will be subjected to  $P_2O_5$  treatment in zone 10. Thereafter the asphalt removed from zone 10 through line 15 will be passed to oxidation zone 12 wherein a treatment similar to that applied in oxidation zone 11 will be employed. In this case the final asphalt product will be withdrawn from line 17.

To exemplify the operability and utility of the process described, the following examples are presented, showing the properties of asphalts obtainable.

#### EXAMPLE I

As typical of the asphalts obtained by the conventional reduction of residual oils a Venezuelan crude oil was subjected to vacuum reduction providing an asphalt of the following properties:

Table I.—Vacuum reduced asphalt

|                                           |      |      |
|-------------------------------------------|------|------|
| Flash point (Cleveland open cup).....     | ° F. | 485  |
| Softening point (ring and ball).....      | ° F. | 90   |
| Penetration at 77° F., 100 grams, 5 sec.  | mm.  | 300+ |
| 10                                        |      |      |
| Penetration at 32° F., 200 grams, 60 sec. | mm.  | 95   |
| 10                                        |      |      |
| Penetration at 115° F., 50 grams, 5 sec.  | mm.  | 300+ |
| 10                                        |      |      |
| Ductility at 77° F., cm.                  |      | 125  |
| Fural viscosity at 210° F., seconds       |      | 345  |

After an oxidation treatment as provided by air blowing, an asphalt of the character identified in Table I has the following typical properties provided by different degrees of oxidation A, B and C.

Table II.—Oxidized reduced asphalt

|                                            | A    | B    | C    |
|--------------------------------------------|------|------|------|
| Flash Point (Cleveland Open Cup), ° F..... | 530  | 510  | 555  |
| Softening Point (Ring and Ball), ° F.....  | 195  | 226  | 291  |
| Penetration at 77° F./100 gms./5 sec.....  | 29   | 16   | 5    |
| Penetration at 32° F./200 gms./60 sec..... | 18   | 11   | 2    |
| Penetration at 115° F./50 gms./5 sec.....  | 45   | 31   | 6    |
| Ductility at 77° F., cm.....               | 3.5  | 2.5  | 0    |
| P. T. S. X 100.....                        | 1.22 | 1.14 | 1.13 |

As indicated by this example, asphalts obtained by the oxidation of residual oils are characterized by high temperature susceptibility. The asphalts are relatively brittle, possess poor ductility and are otherwise unsuitable for application such as the lining of irrigation canals.

#### EXAMPLE II

The residual oil identified in Table I was subjected to  $P_2O_5$  treatment in the absence of air at a temperature of  $450^{\circ} F.$  Various quantities of  $P_2O_5$ , reported in weight per cent, were employed. The residual oil and  $P_2O_5$  were stirred in a closed vessel, while passing a flow of nitrogen through the mixture to completely exclude the presence of air. The resulting asphalt possessed the following properties:

Table III.—Residual oil  $P_2O_5$  treated in absence of oxygen

| Weight Percent $P_2O_5$ Treat.                      | 2%   | 3%   | 4.5% |
|-----------------------------------------------------|------|------|------|
| Flash Point (Cleveland Open Cup), $^{\circ} F.$     | 550  | 535  | 525  |
| Softening Point (Ring and Ball), $^{\circ} F.$      | 192  | 225  | 231  |
| Penetration at $77^{\circ} F.$ /100 gms./5 sec.     | 60   | 55   | 34   |
| Penetration at $32^{\circ} F.$ /200 gms./60 sec.    | 42   | 36   | 27   |
| Penetration at $115^{\circ} F.$ /50 gms./5 sec.     | 110  | 90   | 47   |
| Ductility at $77^{\circ} F.$ , cm.                  | 6    | 4    | 2.5  |
| Penetration Temperature Susceptibility $\times 100$ | .978 | .787 | .673 |

In considering this data, it is significant that the  $P_2O_5$  treatment in the absence of oxygen resulted in an increase in the softening point of the asphalt in proportion to the amount of  $P_2O_5$  employed. To this extent, the treatment has a similar effect to oxidation as illustrated by Table II. However, unlike oxidation, the  $P_2O_5$  treatment provides asphalts of lower temperature susceptibility and greater ductility at comparable softening points. This is well demonstrated by a comparison of Table II and Table III, showing the properties of three asphalts of approximately the same softening point as obtained by oxidation and  $P_2O_5$  treatment respectively.

To further illustrate the effect of reacting  $P_2O_5$  in the absence of air other data employing asphalts and blends of asphalts from other crude sources were obtained:

Table IV

|                                           | Vacuum Reduced Talco Crude, $110^{\circ} F.$ S. P., 1.156 Furol Vis. See at $210^{\circ} F.$ | Talco Blend of 21/30 Pen. Straight Reduced Asphalt with Phenol Extract, 1,079 Furol Vis. See. at $210^{\circ} F.$ | Talco Blend of 21/30 Pen. Straight Reduced Asphalt with Phenol Extract, 836 Furol Vis. See. at $210^{\circ} F.$ |
|-------------------------------------------|----------------------------------------------------------------------------------------------|-------------------------------------------------------------------------------------------------------------------|-----------------------------------------------------------------------------------------------------------------|
| Percent $P_2O_5$                          | 1.2                                                                                          | 2½                                                                                                                | 2½                                                                                                              |
| Flash (Cleveland Open Cup), $^{\circ} F.$ |                                                                                              | 525                                                                                                               | 530                                                                                                             |
| S. P. (Ring and Ball), $^{\circ} F.$      | 174                                                                                          | 187                                                                                                               | 205                                                                                                             |
| Pen., $77^{\circ} F.$ /100 gms./5 sec.    | 47                                                                                           | 57                                                                                                                | 53                                                                                                              |
| Pen., $32^{\circ} F.$ /200 gms./60 sec.   | 29                                                                                           | 32                                                                                                                | 31                                                                                                              |
| Pen., $115^{\circ} F.$ /50 gms./5 sec.    | 85                                                                                           | 101                                                                                                               | 80                                                                                                              |
| Duct., $77^{\circ} F.$ , cm.              | 5½                                                                                           | 5½                                                                                                                | 3½                                                                                                              |
| P. T. S. $\times 100$                     | 1.27                                                                                         | 1.04                                                                                                              | .92                                                                                                             |

In the data shown, the blended asphalts were prepared by utilizing the phenol extract of lubricating oil to provide asphalts of the indicated properties. These data reveal that crude source, composition, viscosity, etc., may influence, but do not prevent the reaction of  $P_2O_5$  in the absence of air with the asphalt. The properties shown above indicate that the catalytically prepared

asphalts have lower temperature susceptibility, are more ductile and are better than those that may be produced by blending or vacuum reduction.

#### EXAMPLE III

As indicated, the treatment of a residual oil or an asphalt with  $P_2O_5$  in accordance with this invention, provides asphalts having properties not obtainable by an oxidation treatment. To obtain the full benefits of this invention, therefore,  $P_2O_5$  treatment must be conducted so as to exclude air to eliminate oxidation effects occurring simultaneously with the  $P_2O_5$  treatment. The deleterious effects caused by the presence of oxygen while treating with  $P_2O_5$  are shown by the following data:

Table V.—Talco flux  $-110^{\circ} F.$  S. P. 1.156 Furol Vis. at  $210^{\circ} F.$

| Percent $P_2O_5$                        | No Air Present |      | Air Present |      |
|-----------------------------------------|----------------|------|-------------|------|
|                                         | 0.7            | 1.94 | 0.7         | 1.96 |
| S. P. (Ring and Ball), $^{\circ} F.$    | 130            | 164  | 127         | 164  |
| Pen., $77^{\circ} F.$ /100 gms./5 sec.  | 80             | 60   | 85          | 54   |
| Pen., $32^{\circ} F.$ /200 gms./60 sec. | 28             | 30   | 34          | 27   |
| Duct., $77^{\circ} F.$ , cm.            | 67             | 10   | 60          | 5.4  |
| P. T. S. $\times 100$                   | 1.89           | 1.29 | 1.95        | 1.35 |

As demonstrated by this data, at the same  $P_2O_5$  level and the same S. P. level, when reacting with  $P_2O_5$  in the presence of air the ductility of final product is lower than when air is excluded. Also, the low temperature properties of the final product are improved when air is excluded.

#### EXAMPLE IV

As demonstrated, oxidation during  $P_2O_5$  treatment is to be avoided to prevent degradation in the properties of the asphalt obtained. However, carefully controlled and relatively mild oxidation may in some cases advantageously be employed prior to the  $P_2O_5$  treatment. This permits a reduction in the amount of  $P_2O_5$  required to obtain an asphalt of a particular softening point, while still providing an asphalt of substantially the same quality. The asphalt obtained is superior to asphalt produced by oxidation alone or produced by  $P_2O_5$  treatment conducted in the presence of air. This process is particularly adapted for improving the properties of an asphalt which has been oxidized.

These principles are illustrated in Table VI below, showing the effect of  $P_2O_5$  treating an asphalt, in the absence of oxygen, after submitting the asphalt to a prior oxidation treatment conducted so as to only partially raise the softening point toward the desired value. The air blowing or oxidation treatment employed consisted of passing 30.5 cu. ft. of air/minute/ton through the asphalt for two hours at  $450^{\circ} F.$  The subsequent  $P_2O_5$  treatment employed  $1\frac{1}{2}$  weight percent  $P_2O_5$ .

Table VI.—Oxidation followed by  $P_2O_5$  treatment

|                                                 | Venezuelan Flux | Air Blown | $P_2O_5$ Treatment of Air Blown Flux |
|-------------------------------------------------|-----------------|-----------|--------------------------------------|
| Flash Point (Cleveland Open Cup), $^{\circ} F.$ | 485             | 540       | 540                                  |
| Softening Point (Ring and Ball), $^{\circ} F.$  | 90              | 105       | 198                                  |
| Pen., $77^{\circ} F.$ /100 gms./5 sec.          | 300+            | 173       | 53                                   |
| Pen., $32^{\circ} F.$ /200 gms./60 sec.         | 95              | 51        | 31                                   |
| Pen., $115^{\circ} F.$ /50 gms./5 sec.          | 300+            | 300+      | 91                                   |
| Duct., $77^{\circ} F.$ , cm.                    |                 | 4.5       | 3.5                                  |

7  
EXAMPLE V

It is sometimes desirable to utilize an oxidation treatment as a finishing step after a prior  $P_2O_5$  treatment conducted in the absence of oxygen. This permits an increase in the softening point of the  $P_2O_5$  treated asphalt without causing any substantial degradation in the other properties of the asphalt. Again this process permits obtaining an asphalt of a desired softening point and other properties while minimizing the quantity of  $P_2O_5$  required.

Table VII shows the properties of an asphalt which was subjected to oxidation treatment after a  $P_2O_5$  treat in the absence of oxygen. The initial feed material was a Venezuelan flux which was raised to a softening point of 232° F. by treatment with  $P_2O_5$  in the absence of oxygen. Thereafter this asphalt was oxidized to a final softening point of 250° F. The inspections of this asphalt were as follows:

| Table VII.—Oxidation of $P_2O_5$ treated asphalt |          |
|--------------------------------------------------|----------|
| Flash (Cleveland open cup)                       | ° F. 540 |
| Softening point (ring and ball)                  | ° F. 250 |
| Penetration at 77° F./100 gms./5 sec.            | 42       |
| Penetration at 32° F./200 gms./60 sec.           | 29       |
| Penetration at 115° F./50 gms./5 sec.            | 60       |
| Ductility at 77° F., cm.                         | 2        |
| P. T. S. $\times 100$                            | 0.74     |

The relatively high ductility and low temperature susceptibility of this high softening point asphalt are significant.

## EXAMPLE VI

As brought out by the preceding examples, asphalts of desired properties are obtained by a  $P_2O_5$  treatment in the absence of air. In particular such asphalts are noted by high softening point, low temperature susceptibility, and high ductility. However, other properties of these asphalts are notable. For example, it has been found that cut-back asphalts prepared by dilution of an asphalt with an agent such as naphtha are resistant to gellation. "Gelling" of an asphalt is notable on storage, causing a substantial increase in the viscosity of the asphalt, making use of the asphalt difficult or impossible. The gelling properties of an asphalt prepared by air blowing a Venezuelan stock and by  $P_2O_5$  treating this stock are shown in the following table:

8  
Table VIIICUTBACK ASPHALT—VISCOSITY INCREASE  
[45% asphalt by weight; 55% naphtha by weight]

|    |                                                                     |                                                                                                 |
|----|---------------------------------------------------------------------|-------------------------------------------------------------------------------------------------|
| 5  | 220/235 Venezuelan Stock Prepared by air blowing; Pen. at 32° F.=11 | 210 S. P. Venezuelan Stock Prepared by $P_2O_5$ Treatment of Venezuelan Flux; Pen. at 32° F.=39 |
| 10 | 1 day 60,000+ cps; gelled immediately                               | 31 cps.                                                                                         |
|    | 4 days                                                              | 34 cps.                                                                                         |
|    | 11 days                                                             | 37 cps.                                                                                         |
|    | 13 days                                                             | 41 cps.                                                                                         |
|    | 19 days                                                             | 44 cps.                                                                                         |

The  $P_2O_5$  treated asphalt was prepared by treating the identified flux with 2.2 wt. percent of  $P_2O_5$  with agitation in the absence of air for 5 hours at 450° F. As shown by this data, the  $P_2O_5$  treated asphalt was not subject to gellation.

What is claimed is:

1. A process for treating residual oils comprising adding about 0.1 to 5% by weight of  $P_2O_5$  to said residual oil and agitating said mixture in the absence of free oxygen at a temperature of about 300° to 550° F.
2. In the treatment of residual oils and asphalts with  $P_2O_5$ , the improvement which comprises adding about 0.1 to 5 weight percent of  $P_2O_5$  to the said composition to be treated and thereafter agitating this mixture in the absence of free oxygen at a temperature of about 300° to 550° F.
3. A process for producing asphalt from a residual oil in which the residual oil is mixed with about 0.1 to 5 weight percent of  $P_2O_5$  in the absence of free oxygen at a temperature of about 300° to 550° F.
4. The process defined by claim 3 in which the said residual oil is oxidized prior to the said treatment with  $P_2O_5$ .
5. The process defined by claim 3 in which the said treated mixture is oxidized after the said treatment with  $P_2O_5$ .

45  
References Cited in the file of this patent

## UNITED STATES PATENTS

| Number    | Name        | Date         |
|-----------|-------------|--------------|
| 2,179,208 | Burk et al. | Nov. 7, 1939 |
| 2,281,728 | Thelen      | May 5, 1942  |
| 2,450,756 | Hoiberg     | Oct. 5, 1948 |